

# United States Patent Office.

NATHAN WASHBURN, OF WORCESTER, MASSACHUSETTS.

Letters Patent No. 92,676, dated July 13, 1869.

## IMPROVED MODE OF REPAIRING PLUMBAGO CRUCIBLES USED IN MELTING STEEL.

The Schedule referred to in these Letters Patent and making part of the same

To all persons to whom these presents may come:

Be it known that I, NATHAN WASHBURN, of the city and county of Worcester, and State of Massachusetts, have made a new and useful Invention, having reference to the Repairing of Plumbago Crucibles, as used in furnaces for the making of cast-steel; and I do hereby declare the same to be fully described in the following specification.

It is well known that a crucible of the kind mentioned will not, generally speaking, stand more than two or three heats of the furnace, before becoming so injured as to be rendered unfit for further use.

Attempts have been made to repair such crucibles, by dipping them in a fluid-composition of plumbago, mica, and clay, and a patent has recently been taken out for such, by William F. Sherman, it being numbered 87,075; but it has been found, in practice, that this process of repair, though often useful, cannot be depended on, both on account of the uneven thickness in which the crucible is left after having been dipped, and the fact that spaces containing air will be formed in the coating, or between it and the surface to which it may be applied. On heating the crucible, the air will be expanded, and cause the coating to scale off or break away from the crucible.

A crucible, after having been charged, and submitted to the action of the powerful heat of a steel-melting furnace, generally becomes more or less warped, as well as cut away, so as to be of an uneven thickness; that is to say, it will be reduced more in some places or parts than in others, so that when the restoration is attempted to be effected by the dipping-process, the crucible, after the carrying out of the same, remains of an uneven thickness.

It is very important that the proper thickness of the crucible should be preserved, in order that the metal or the flux used while the crucible is being heated, may not cut through it.

These plumbago crucibles, as ordinarily mended, have been a source of great expense to the makers of cast-steel, for as two or three heats of the furnace, at the most, would generally destroy them, and as they usually cost from three to four dollars a piece, the loss per ton, of steel, has been equal to forty dollars.

Steel-makers generally reckon that it costs them, for every pound of steel produced, about two cents for the crucible. Therefore, it will be seen that any mode of repairing these crucibles, by which they will be rendered capable of withstanding, for a longer period, the heat of the furnace, must be a great gain to the maker of steel.

My method of repairing enables a crucible to be used a great number of times; I may state almost an indefinite number. Practice has proved this, as in-

stead of simply applying to the crucible a coating of even thickness, by the process of dipping, thereby leaving the injured crucible of an uneven thickness, I restore the crucible to its normal thickness, and expel from the repairing-composition any and all the air which would operate to cause it to scale off under the heat of the furnace.

A crucible that had been subjected to the dipping-process and condemned, I have treated by my method, and used it in several heats of the furnace, thus utilizing it to great advantage.

In running twenty-four crucibles, and melting thereby three tons of steel, I find the saving, by my method of repairing, is about seventy-five dollars, and with reference to the dipping-process, I save about fifty dollars, the saving by the dipping-process not exceeding twenty-five dollars.

These results I mention, to exhibit the vast utility of my invention, and the great saving of expense to the manufacturer of steel.

In carrying out my said invention, I usually employ a composition consisting of Stourbridge clay, fire-brick, and graphite, in equal, or about equal quantities,

These ingredients, after having been ground to a fine powder, are to be mixed into a paste or mortar, with water. This mortar is next to be plastered on the surface or parts thereof of the crucible required to be thickened.

After this has been done, the mortar so put on, and while it may be in the process of setting or hardening, should be rubbed, beaten, and worked, by means of a spatula, or other proper implement, so as to thoroughly drive from it any air or air-bubbles, and compress it, and finally polish or reduce its outer surface to a very smooth state; the smoother the surface the better it will withstand the heat.

The dipping-process leaves the surface rough and uneven, and thus renders it more susceptible of injury by the heat of the furnace.

I make no claim to mere dipping a crucible in a thin solution of plumbago, mica, and clay, or the equivalent thereof, for reparation of it.

What I claim as my invention, is—

The employment of a composition, as set forth, or its equivalent, in the form of a mortar, and plastering it on the injured crucible, and working it when thereon, so as to expel the air from the said repairing-medium, and bring the crucible to its normal or required thickness, and impart to it a smooth outer surface, as specified.

N. WASHBURN.

Witnesses:

R. H. EDDY,  
S. N. PIPER.